

1

**3,551,271**  
**NONWOVEN FABRICS CONTAINING**  
**HETEROFILAMENTS**

Gwilym G. Thomas, Panteg, and Christopher R. Sissons, Raglan, England, assignors to British Nylon Spinners Limited, Pontypool, England  
 No Drawing. Continuation of application Ser. No. 473,824, July 21, 1965. This application July 15, 1969, Ser. No. 847,499  
 Claims priority, application Great Britain, July 30, 1964, 30,442/64

Int. Cl. D04h 1/04, 1/54, 3/00  
 U.S. Cl. 161—150      5 Claims

### ABSTRACT OF THE DISCLOSURE

A non-woven fabric is made by forming a web containing at least 5% by weight heterofilaments comprising at least two components at least one of which is an elastomer and at least one of which is potentially adhesive, and subsequently activating the adhesive component to bond the structure at the filament cross-over points. Preferably the elastomeric and potentially adhesive component are the same component.

### DISCLOSURE

This application is a continuation of Ser. No. 473,824, filed July 21, 1965, and now abandoned.

This invention relates to nonwoven fabrics and to processes for making them.

Nonwoven fabrics as heretofore available have usually suffered from certain property limitations and weaknesses which have tended to restrict their range of applications. Particularly deleterious properties in regard to the employment of nonwoven fabrics in the making, for example, of articles of apparel, have been their general stiff, board-like character and their poor drapability. A number of proposals have been advanced in an attempt to ameliorate those properties, but, generally speaking, the improvements can be effected only by sacrificing strength in the fabric, and this lack of strength may militate against the acceptance of the fabric for certain end uses.

In applications, Ser. No. 346,752 filed Feb. 24, 1964 and Ser. No. 342,300, filed Feb. 4, 1964, both abandoned, there is described and claimed inter alia nonwoven fabrics which exhibit in combination an adequate drapability and a good tensile strength. In broad and somewhat simplified terms, the advantageous combination of properties possessed by the nonwoven fabrics of the aforementioned applications is owed to our discovery of the efficacy of incorporating in the fibrous webs, from which the fabrics are devised, at least a proportion of composite filaments, of which heterofilaments, that is to say, unitary filaments, consisting of two or more polymeric components contiguous and adherent to one another continuously along the length of the filament are a particular advantageous type.

This invention is based on our discovery of the utility of a certain type of heterofilament in providing nonwoven fabrics which posses not only tensile strength of the same order of magnitude as the fabrics provided by our previously mentioned applications, but, in addition, have a superior drapability, flexibility, crease-resistance properties and conformability.

Accordingly, the nonwoven fabrics of this invention comprise fibrous webs containing at least five percent heterofilaments consisting of two or more components, at least one of which is an elastomer, fibres in the fibrous webs being bonded together at points where they cross-

2

over and contact one another by the adhesive characteristics of a potentially adhesive component of said heterofilaments.

For convenience of discussion we will consider the heterofilament to consist only of two components although it will be understood that the filaments may, if desired, have more than two components. In the two component heterofilaments one or both of the components may be an elastomer. The heterofilaments containing at least one elastomeric component will be referred to herein as elastomeric heterofilaments. For convenience in this specification the non-elastomeric component will be referred to as a "hard" component.

By the expression "potentially adhesive component" as used in this specification and the claiming clauses appended hereto we mean a component the adhesive characteristics of which can be developed without sensibly affecting the other component of the heterofilament.

In the heterofilaments which contain one hard and one elastomeric component, either may be the potentially adhesive component although in certain respects discussed more fully hereinafter it is desirable that the elastomeric component should be the potentially adhesive component.

The terms "filament" and "fibre" are used in this specification and in the claiming clauses appended hereto in the generic sense and include continuous filaments, and staple fibres including flock.

The incorporation in the fibrous web from which the fabrics are derived of heterofilaments possessing at least one elastomeric component endows the fabric with resilience and flexibility, properties which are reflected in the good drapability, crease-resistance and conformability of the fabrics.

Drapability is measured by determining the length of fabric (the bending length) which is necessary to cause the fabric to bend from the horizontal plane when under no constraint to such an extent as to contact a declining angle of 41.5° of slope from the point of departure of contact.

Conformability is largely a subjective property which we find convenient for expressing the ability of the fabric to give and yield in adopting a particular configuration. In relation to the application of the fabrics as articles of apparel, it is important that they should have a good conformability.

Flexural rigidity is a measure of the fabric stiffness or flexibility and is related to the quality of stiffness that is appreciated on handling the fabric, and its measurement involves determining the length of fabric which is necessary to cause the fabric to bend from the horizontal plane when under no constraint to such an extent as to contact a plane surface inclined at an angle of 41.5° to the horizontal. The procedure is fully described in British standard specification No. 3,356/1961. Briefly stated, it comprises placing a one inch wide strip of the fabric upon a horizontal surface, one end of which abuts against the top end of a 41.5° inclined plane. The test sample is placed with its narrow edge at the juncture of the horizontal and inclined surfaces. It is then moved forward over the edge between the two surfaces until the free end bends over and contacts the inclined surface. The length of the arc (cantilever length) between the point of departure from the horizontal surface and the point of contact with the inclined surface is measured and this is the bending length (in abbreviated form represented by B.L.). The flexural rigidity can then be evaluated from the formula:

$$\text{Flexural rigidity} = \text{weight per unit length} \times \text{B.L.}^3 \times k$$

The advantageous properties discussed above are most manifest when the potentially adhesive component is an elastomeric component of the heterofilament, for then,

the bonds formed at points of contact and cross-over of fibres in the fibrous web are elastomeric in character and consequently the fabric has a maximum degree of lateral freedom and flexibility in three dimensions.

Although we have discussed the advantageous properties of the nonwoven fabrics of this invention in relation to the use of a particular type of heterofilament (elastomeric heterofilament), the fact that the heterofilaments provide the fibrous web with a built-in-binding action which is owed to the potentially adhesive component thereof, is also of significance in the development of those properties, and, perhaps more importantly, provides the fabric with good dimensional stability and adequate tensile strength without any sacrifice of the desirable low fabric density.

The nonwoven fabrics of this invention combine together the properties of drapability, flexibility, and conformability with good dimensional stability and tensile strength.

The introduction of resilience and flexibility in the fabrics by using heterofilaments which contain only one elastomeric component successfully overcomes difficulties which we have experienced in attempting to import those properties into fabrics by using elastic homofilaments. Among the difficulties which we have found associated with this latter method are, the difficulties of web formation, the tendency of the elastic fibres to migrate throughout the web during and subsequent to processing, and the trouble experienced in attempting to form a coherent structure by needle-punching. That these difficulties are largely obviated when the elastic fibre is incorporated in the web and resulting fabric as one component of a heterofilament can be attributed to the presence of the other component and its role in, for example, restraining the elastomeric component which is held along its length in association with that component.

In selecting the components for the heterofilaments attention should be paid to their compatibility one with another and also to their ability to adhere together to form a unitary filament.

The heterofilaments may be prepared by any of the well-known processes. Thus melts, or solutions, of the polymeric components may be extruded simultaneously through an orifice in sheath and core or side-by-side relationship, or the components may be extruded through separate orifices using known apparatus and subsequently brought into adhering contact with one another whilst they are still in a tacky condition to form a unitary filament.

As the hard component which may be present in the heterofilaments there are called into question synthetic condensation polymers such, for example, as polyesters, polyamides, polyurethanes, polyureas, and polycarbonates, addition type polymers such as the polyhydrocarbons, and those made from ethylenically unsaturated monomers such, for example, as vinyl chloride, vinylidene chloride, vinyl acetate, acrylonitrile and their copolymers.

The term "elastomer" as used herein has the meaning conventionally given to the term in the art.

Suitable elastomers for use in this invention may be found in many classes of fibre-forming polymer. The elastomer may, for example, be a segmented (block copolymer) elastomer, of which, as examples, there may be mentioned the following:

N-substituted copolyamides containing from 15-34 percent of N-substitution and prepared by the reaction of a lactam of an omega-amino carboxylic acid with N-substituted amino-carboxylic acid containing more than 7 carbon atoms; N-substituted polyamides containing from 15-38 percent of N-substitution and prepared by the reaction of an N,N'-disubstituted aliphatic secondary diamine, a dibasic carboxylic acid containing at least 5 carbon atoms in the chain and a lactam of an omega-amino carboxylic acid containing 7-20 ring members or by the reaction of an N mono substituted aliphatic di-

amine, a dibasic carboxylic acid containing at least 5 carbon atoms in the chain and a lactam of an omega-amino carboxylic acid containing 7-20 ring members.

N-alkyl-substituted copolyamides as described in British Patent No. 692,069; and

5 Polyester-urethanes generally, but in particular those and made from a hydroxyl-terminated copolyester of molecular weight greater than 1500, a dihydric alcohol and an aliphatic or cycloaliphatic diisocyanate, the diisocyanate not being present in a molar excess at any time during the making of the polyurethane.

10 Suitable elastomers may also be formed using the fibre-forming addition polymers, for example, copolymers of butadiene/acrylonitrile, butadiene/styrene, and butadiene/2-vinyl pyridine, polychlorobutadiene and copolymers of isobutylene with small proportions of butadiene.

15 Examples of two component heterofilaments, containing both a hard and an elastomeric component are those characterised by their ability to crimp spontaneously at drawing. Such heterofilaments are characterised by a crimp frequency of at least 10 crimps per inch.

20 A variety of methods are available by which the nonwoven fabrics of this invention may be made, and the method chosen will depend to a very large extent upon the particular kind of fabric within the general class desired. Common to all the available methods is the initial step of fabricating a fibrous web.

25 The fibrous web itself may be formed by any of a number of known techniques for depositing or arranging fibres in a web.

30 These techniques include carding, garnetting, air-laying and paper-making techniques for the fabrication of staple fibres webs. Continuous filament webs may conveniently be prepared by drawing off the filaments directly from a spinning unit, or they may be formed from a package or other storage device for yarn already spun. Continuous filament yarn webs, that is to say, webs in which the filaments are present as multifilaments may conveniently be prepared in a process wherein freshly spun filaments are subjected to the action of a high velocity turbulent fluid jet which attenuates and orients the filaments and intermingles them to form a twistless yarn, which yarn is forwarded by the fluid jet and deposited on a receiving surface in a random loopy manner.

35 40 45 In one method of making fabrics in accordance with this invention the fibrous web is subjected to a heat and pressure treatment, for example, by passage between the nip of heated calender rollers, whereby the potentially adhesive component is activated i.e. rendered adhesive.

50 In another method of making the fabrics at least the heterofilaments in the fibrous web are crimped or, if they are already crimped, further crimped, prior to or during the treatment to which the web is subjected in order to activate the potentially adhesive component of the heterofilaments.

55 Heterofilaments may be crimped by exposing the fibrous web containing them to a suitable shrinking treatment. The shrinkage of the heterofilaments in order to effect crimping may be carried out by the use of any suitable shrinking agent. Shrinking may, for example, be carried out by heating by various means, as by the application of hot aqueous media (for example, hot or boiling water, and steam including pressurised steam), oil, hot air or other hot gaseous or liquid media chemically inert to the polymer components of the heterofilaments. Alternatively, or in addition, the heterofilaments may be crimped, or further crimped, by exposing the fibrous web to the action of a swelling agent for one component of the heterofilaments.

60 65 70 75 70 Whether crimp be effected by a physical or chemical treatment we frequently find it convenient to activate the potentially adhesive component, thereby bonding together fibres of the web where they cross-over or contact one another, in the same treatment. Thus, crimp and activation may be effected by subjecting the fibrous web to a

heat treatment in which the temperature exceeds the softening point of the potentially adhesive component. Examples of heterofilaments which can be crimped and activated in this manner and the conditions under which these steps can occur are shown in the table below:

|                                                              | Potentially adhesive component                              | Temp. °C. |
|--------------------------------------------------------------|-------------------------------------------------------------|-----------|
| Poly(omega-aminoundecanoic acid)...                          | NN'-di-isobutyl hexamethylene sebacamide/poly(capro amide). | 160       |
| Maranyl L.A. (Identified in Example A polyester urethane 2). |                                                             | 170       |

When the potentially adhesive component of the heterofilament is such that it can be chemically activated the crimping and activation steps may be accomplished in the same chemical treatment. Such a chemical treatment may conveniently be adopted for heterofilaments consisting, for example, of various proportions by weight for example, equal quantities of Maranyl L.A., which is a polyamide copolymer identified in Example 2, as the hard component, and a polyester urethane as the elastomeric, and also the potentially adhesive, component, the two components being arranged in a side-by-side relationship. Such heterofilaments can be crimped, and the elastomer component rendered adhesive, by treating the fibrous web containing the heterofilament at room temperature in a bath of dimethylformamide which can be considered as a selective solvent for the elastomer component.

In all circumstances in which crimping and activation are achieved in separate treatments, the fibrous web, after crimp has been developed in fibres therein, is subjected to a further treatment to activate the potentially adhesive component thereby bonding together fibres of the web where they cross-over or contact one another. Bonding in this manner can be accomplished in a variety of ways and in any particular instance the method used is, to a large extent, dependent on the nature of the potentially adhesive component and also that of the other component of the heterofilament. Where the potentially adhesive component has a lower softening point than the other, it may conveniently be made adhesive by subjecting the web to a heat treatment which may, for example, be achieved by dry heat, as by passing hot air through the web or by heating it in an electric oven, or by treating the web with moist heat as by the use of moist air, hot water or steam. Other possible methods of heat activation include exposing the web to radiation, for example, infrared radiation of a suitable intensity and duration. When the potentially adhesive component is capable of being activated chemically, activation may be achieved by an appropriate chemical treatment.

Whenever crimp is developed in the heterofilaments of the fibrous web, the resulting fabric has a superior bulk or loft, a better developed resiliency and a more open structure than a fabric made from the fibrous web under conditions, for example subjecting the web to a simultaneous heat and pressure treatment, wherein no crimp is developed.

A fabric possessing a compact porous structure and suitable for use in the making of a synthetic leather material may be obtained from the bulky resilient fabric by applying a pressure to the latter within a short interval of time after the fibre bonds have been formed i.e. while they are still in an adhesive condition. Under the applied pressure the crimped fibres are deformed in a manner somewhat analogous to the depression of a helical spring and a myriad of small pores which confer "breathability" on the resulting fabric are preserved therein.

It is only necessary that the fibrous web contain five percent heterofilaments, although we prefer that they be present in an amount of twenty percent or more, and other fibres which are inert or substantially so to the activation treatment to which the web is subjected may be employed

as a blend with the heterofilaments. Although those other fibres must be inert to the activation treatment they may be potentially crimpable, in which event they may be crimped in any treatment to which the web is subjected to crimp, or further crimp, the heterofilaments therein. Depending upon the particular desiderata sought in the fabric, the percentage of heterofilaments present in the fibrous web may be varied widely.

The nonwoven fabrics find applications in many diverse fields, but they are particularly well adapted for end uses which demand a fabric possessing a good drape, flexibility, crease-resistance and conformability combined with an adequate tensile strength and air-permeability, uses wherein the advantageous properties of the present fabrics are utilised to the full. The fabrics are, for example, suitable for a number of applications as articles of apparel.

By way of illustration, but not by way of limiting the invention there will now be given the following specific examples.

#### Example 1

In the heterofilament used in this example, the elastomeric component was an N-substituted polyamide of the type prepared by heating together 192 gms. of N,N'-di-isobutyl hexamethylene diamine, 162 gms. of sebacic acid, and 814 gms. of caprolactam in the presence of 16 gms. omega-amino-undecanoic acid, 1 gm. of orthophosphoric acid and 50 mls. of water as polymerisation catalysts. The resulting polyamide in which approximately 25 percent of the nitrogen atoms carried isobutyl substituents had an inherent viscosity of 0.6, and a softening point of 160° C. The hard component of the heterofilament was nylon 11 having a softening point of 190° C. and an inherent viscosity of 0.63.

A monofilament comprising the above two components arranged in a side-by-side relationship was made by melting under pressure in a spinning machine a sintered rod consisting of equal parts of the two components the spinning machine being adapted to force the molten polymers at a temperature of 240° C. through an undivided filter pack and then extruding the polymers through an orifice contained in a spinneret plate. The extruded monofilament was dusted with talc and then wound onto a bobbin at a rate of 400 feet per minute.

The monofilament was subsequently cold drawn at ambient temperature at a draw ratio of 4:1. The filament crimped spontaneously on relaxing from the drawing tension and had a denier of 15 and a crimp frequently of 2 per inch.

18 gms. of three inch staple fibres formed from the crimped heterofilament were carded on a Shirley miniature card and the laps so formed laid on top of one another with successive laps disposed at an angle of 90° with respect to the previous lap so forming a cross-laid web having a weight of 9 ounces per square yard. A 5" x 4 1/2" portion of this cross-laid web was placed between the heated plates of a hot press maintained at a temperature of 160° C. and therein subjected to a pressure of 300 p.s.i. for a period of 1 1/4 minutes.

The resulting fabric was in the form of a thin sheet.

On examining the fabric under the microscope it was observed that in consequence of the temperature and the applied pressure the adhesive characteristics of the elastomer component of the heterofilament had been developed and refined bonds had formed at the points of contact and cross-over of adjacent fibres. Despite the activation treatment to which the web had been subjected the elastomeric component remained in contiguous association with the poly(omega-undecanoic acid) component which retained its fibrous form. The absence, of any spread of the potentially adhesive, that is to say, the elastomeric component, throughout the structure and the refined nature of the bonds formed resulted in preservation of substantially all the interstitial spaces between fibres, and gave the resulting fabric a porous air-permeable structure.

On examining the fabric under the microscope it was observed that in consequence of the temperature and the applied pressure the adhesive characteristics of the elastomer component of the heterofilament had been developed and refined bonds had formed at the points of contact and cross-over of adjacent fibres. Despite the activation treatment to which the web had been subjected the elastomeric component remained in contiguous association with the poly(omega-undecanoic acid) component which retained its fibrous form. The absence, of any spread of the potentially adhesive, that is to say, the elastomeric component, throughout the structure and the refined nature of the bonds formed resulted in preservation of substantially all the interstitial spaces between fibres, and gave the resulting fabric a porous air-permeable structure.

The fabric was a drapable material having a texture simulating to a certain degree that of a woven fabric. It had the physical properties shown in the table which follows:

|                             |       |
|-----------------------------|-------|
| Density, gm./cc.            | 0.5   |
| Mean bending length, cms.   | 4.25  |
| Flexural rigidity, mgm. cm. | 2,350 |

Since the fabric had a homogeneous structure, in the sense that, it consisted entirely of fibres all of which were selected from the same chemical classification i.e. all the fibres had the same functional groups, it was readily dyed with only one dyestuff. To produce a leather-like material the fabric could be coated, for example, with a polyurethane, and dried. A leather-like grain could be imprinted on the coated surface of the dyed fabric by pressing the surface with a patterned heated embossing plate.

The influence of the elastomeric component of the heterofilament in endowing the fabric with resilience and flexibility, properties which find expression in the good drapability, flexibility, crease-resistance and tensile strength which the fabric possesses, can conveniently be illustrated by a comparison of the measured physical properties of the fabric with a fabric derived from a fibrous web consisting of heterofilaments which contain two components, none of which are elastomeric. Such a fabric may be prepared in the following manner:

A quantity of two and a half inch 15 denier staple fibres formed from heterofilaments consisting of equal proportions by weight of poly(hexamethylene adipamide) and an 80/20 random copolymer of poly(hexamethylene adipamide)/poly(epsilon caprolactam) (nylon 66/66/6), the two components being arranged in a side-by-side relationship, was carded in a Shirley miniature card, and the laps so formed laid on top of each other with successive laps disposed at an angle of 90° with respect to the previous lap so forming a cross-laid web having a weight of 9 ounces per square yard. The web was then placed between the two heated plates of a hot press maintained at a temperature of 230° C. and subjected therein to a pressure of 300 p.s.i. for a period of 1 1/4 minutes. In consequence of the temperature and pressure to which the fibrous web was subjected, the adhesive characteristics of the lower melting point component, i.e. the copolymer component, of the heterofilament were developed, that is to say, it became adhesive thereby causing fibres in contact with one another to stick or fuse together.

The fabric which was strong had a stiff and board-like handle. It had the properties listed in the table below:

poly(hexamethylene adipamide) and poly(hexamethylene sebacamide) sold by Imperial Chemical Industries Limited under the name Maranyl L.A. 29. It had a Vicat softening point of 190° C. and an inherent viscosity of 0.962. The elastomeric component was a polyester urethane. The extruded monofilament was passed through an aspirating jet within which it was acted upon by high velocity air supplied through an inlet in the sidewall of the jet. Toroidal vortices having their axes substantially perpendicular to the mean axis of the filament, are thought to be formed within the jet thereby creating a turbulent zone around the filament which had the effect of whipping the filament from side to side. The filament was forwarded by the blast of air issuing from the jet, to a foraminous receiving surface where it was laid in a random loopy manner in the form of a continuous filament web having a weight of approximately 1 ounce per square yard. A portion (15.7 cms. x 19.4 cms.) of this web weighing 1.1 gms. was placed between two brown paper sheets, each of which had previously been coated with poly(tetrafluoroethylene), and the resulting "sandwich" passed at a rate of 1 foot per minute between the nip of two calendar rollers each four inches in diameter and which exerted a pressure of approximately 100 p.s.i. The temperature of the calendar rolls was of the order of 178° C.

The effect, upon the fibrous web, of the heat and pressure applied in the calendar was to activate the polyester urethane component of the heterofilaments, which became tacky and in this condition bonded together fibres in the fibrous web at points where they cross-over or contact one another.

The bonds which confer upon the fabric dimensional integrity and mechanical strength were elastomeric in character and consequently the fabric possessed a high degree of lateral freedom and flexibility in three dimensions. The excellent drapability, crease-resistance and conformability of the fabric can be attributed to the elastomeric bonds holding the fabric together and to the presence in the heterofilaments of an elastomeric component. Moreover, since the polyester-urethane on activation formed refined bonds, that is to say, there was an absence of blobs, the fibres being cemented together only at points of contact and the polyester urethane over the greater part of the length of the heterofilaments remained in contiguous association with the hard component, the fabric had a porous, air-permeable structure.

Those properties of the nonwoven fabric discussed above find expression in the physical measurements listed in the table which follows:

| Direction          | Properties       |                           |                            |                    |                               |                                        |                                     |
|--------------------|------------------|---------------------------|----------------------------|--------------------|-------------------------------|----------------------------------------|-------------------------------------|
|                    | Density, gm./cc. | Mean bending length, cms. | Flexural rigidity, mgm.cm. | Extension, percent | Tensile strength, kg./gm./cm. | Elastic recovery, 10 percent extension | Work recovery, 10 percent extension |
| Along fabric-----  | 0.3              | 2.0                       | 30                         | 57                 | 443 }                         | 80                                     | 66                                  |
| Across fabric----- | 0.3              | 1.75                      | 21                         | 60                 | 358 }                         |                                        |                                     |

Density—0.45 gm./cc.

Mean bending length—very much greater than 6 cms.

Flexural rigidity—very much greater than 6,500 mg./cm.

It will be observed that the drape of the novel fabric described in this example was at least some 30 percent better than the drape of the fabric derived from the non-elastomeric heterofilaments.

#### Example 2

In this example the two component heterofilament, only one of which component was elastomeric, was melt spun into a monofilament by the method described heretofore in regard to Example 1, the spinning temperature being 300° C. The hard component was a copolymer of

To demonstrate the superior drape, flexibility, crease-resistance and conformability of the nonwoven fabric of this example when compared with a fabric derived from heterofilaments which contained no elastomeric component, a continuous filament web having similar basic weight (1.15 ounces per square yard) as the web described hereinbefore was made by the same method from a heterofilament consisting of poly(epsilon caprolactam) as one component and an 80/20 random copolymer of poly(epsilon caprolactam) and poly(hexamethylene adipamide) as the other. The web was then fused by passage through calender rolls, under identical conditions as before except that the temperature was 200° C., thereby forming a sheet fabric weighing 1.5 ounces per square

yard and having the properties shown in the table which follows:

| Direction           | Properties       |                          |                             |                    |                               |
|---------------------|------------------|--------------------------|-----------------------------|--------------------|-------------------------------|
|                     | Density, gm./cc. | Mean bending length, cm. | Flexural rigidity, mgm./cm. | Extension, percent | Tensile strength, kg./gm./cm. |
| Along fabric -----  | 0.3              | 3.3                      | 184                         | 11                 | 95                            |
| Across fabric ----- | 0.3              | 3.2                      | 166                         | 11                 | 71                            |

On comparing the values listed in this table with the values found for the corresponding properties listed in the preceding table the superiority of the fabric derived from heterofilaments containing an elastomeric component is evident, for it not only had a better drapability, crease-resistance, flexibility and conformability but it also had a much better tensile strength. The combination of all these advantageous properties makes the novel fabric eminently suited for numerous apparel applications.

#### Example 3

A heterofilament having the same components and arrangement thereof as the heterofilament used in Example 2 was extruded as a monofilament in the manner described in Example 1 at a spinning temperature of 200° C. The monofilament which was wound up onto a bobbin at 400 feet/minute had an as-spun denier of 104. It was subsequently cold-drawn at ambient temperature at a draw ratio of 4:1. The filament which had a denier of 20 was cut into  $\frac{3}{8}$ " flock using a Dörstling flock cutting machine.

A quantity of this flock and a quantity of cellulose pulp (weight ratio 3:1) was dispersed by vigorous agitation over a ten minute period, in three litres of water containing a small quantity of Dispersol V.L. (the word Dispersol is a registered trademark). The resulting uniform suspension was filtered over an 8 inch square 100 mesh wire screen to give a uniform coherent web having a weight of  $2\frac{1}{2}$  ounces per square yard, and an excellent wet strength. This web was placed between two poly(tetrafluoroethylene) coated sheets of brown paper so forming a sandwich which was passed at the rate of 1 foot per minute between the nip of a pair of four inch diameter calender rollers maintained at a temperature of 180° C. and exerting a pressure of approximately 100 p.s.i.

As a result of the applied heat and pressure the web experienced considerable area shrinkage and the polyester urethane component of the heterofilament flock became adhesive thereby serving to bond together fibres which came into contact with that component. The fabric, which was considerably more drapable and flexible than a similar fabric derived from a non-elastomer heterofilament, had a weight of four ounces per square yard, an extension of 34 percent and a tensile strength of 83 kg./gm./cm.

#### Example 4

A heterofilament having the same components and arrangement thereof as the heterofilament used in Example 2 was extruded as monofilament in the manner described in Example 1 at a spinning temperature of 200° C. The monofilament which was wound up onto a bobbin at 400 feet/minute had an as-spun denier of 104. It was subsequently drawn at ambient temperature at a draw ratio of 4:1. The filament which had a denier of 20 crimped spontaneously on relaxing from the drawing tension. The crimped 25 denier filament (crimp frequency —12 crimps per inch) was cut into two inch staple, a quantity of which was carded on a Shirley miniature card so as to form a web having a weight of approximately 3 ounces.

This web was then immersed for a period of 30 minutes in dimethylformamide to activate the elastomer compo-

nent of the heterofilament fibres which, in consequence, became adhesive and in that condition bonded together fibres in the web. The ability of the dimethylformamide to activate the elastomer component can be explained on the basis that it is a selective solvent for that component, and as such causes swelling and gelation of the elastomer. In addition to its swelling action the dimethylformamide shrinks the elastomer component thereby further crimping the heterofilament fibres.

The tensile strength and dimensional stability possessed by the resulting nonwoven fabric was owing to the reinforcement of the binding action attributable to the potentially adhesive component by the random interlocking, incurling and/or interlooping resulting from crimp.

The fabric possessed an enhanced bulk and resiliency, a more open appearance, and a lower density as compared with the fabrics of Examples 1 to 3, and this may be attributed, at least in some measure, to the presence in the fabric of crimped filaments and to the absence of any application of pressure in the bonding together of fibres in the fibrous web.

We claim:

1. A nonwoven fabric comprising a fibrous web containing at least five percent, based on the weight of fibres in the web, of heterofilaments consisting of at least two components, at least one of which is an elastomer and which is potentially adhesive, and at least one other component being a hard, non-elastomeric component with fibres in the fibrous web bonded together at points where they cross-over and contact one another by the adhesive characteristics of said elastomeric, potentially adhesive component, said fabric having a bending length of from 1.75 cm. to 4.25 cm. and having a ratio of bending length in centimeters to density in grams per cubic centimeter of from 5.8 to 8.5.

2. A nonwoven fabric as claimed in claim 1 wherein the heterofilaments are crimped.

3. A nonwoven fabric as claimed in claim 2 wherein the heterofilaments have a crimp frequency of at least 10 crimps per inch.

4. A nonwoven fabric as claimed in claim 1 wherein 20 to 50 percent, based on the weight of fibres in the web, of the fibres are heterofilaments and the balance are non-activatable.

5. A nonwoven fabric as claimed in claim 1 wherein 50 to 100 percent, based on the weight of fibres in the web, of the fibres are heterofilaments and the balance, if any, are non-activatable.

#### References Cited

##### UNITED STATES PATENTS

|    |           |         |           |          |
|----|-----------|---------|-----------|----------|
| 65 | 2,774,129 | 12/1956 | Sechrist  | 161—169  |
|    | 3,038,235 | 6/1962  | Zimmerman | 161—175X |
|    | 3,348,993 | 10/1967 | Sissons   | 161—64X  |

ROBERT F. BURNETT, Primary Examiner

R. L. MAY, Assistant Examiner

U.S. Cl. X.R.  
156—306; 161—173